

## 1

2,745,741

## METHOD OF PRODUCING MAGNESIUM BASE ALLOYS

Edward Frederick Emley and William Unsworth, Manchester, England, assignors to Magnesium Elektron Limited, Manchester, England

No Drawing. Application February 13, 1953,  
Serial No. 336,868

Claims priority, application Great Britain October 7, 1952

8 Claims. (Cl. 75—168)

This invention relates to the production of magnesium-base alloys containing thorium, e. g. alloys containing thorium, zinc, and zirconium, in accordance with U. S. Patent No. 2,604,396. These alloys may contain small quantities of rare earth metals, in fact the commercial thorium or thorium compounds used for introducing the required thorium content into the magnesium are frequently contaminated with rare earth metals which are accordingly introduced into the magnesium at the same time. Moreover with reprocessing of scrap the rare earth metal content of such alloys may increase considerably. However, we have found that it is desirable in certain cases for the alloys to be free from rare earth metals. The main object of the present invention therefore is to effect the removal of rare earth metals from magnesium base alloys of the kind in question without appreciable loss of the thorium content. It is already known that fluxes used for the treatment of magnesium base alloys and containing magnesium chloride will cause a reduction of the rare earth metal content by reaction with the magnesium chloride. However, it has heretofore been considered that the thorium content is also reduced by the use of such fluxes due to the reaction of thorium with the magnesium chloride. Thus in the paper entitled "Properties of magnesium-thorium and magnesium-thorium-cerium alloys," Journal of Metals, March 1952, page 287:

"It was observed that the behaviour of thorium in molten magnesium with respect to reaction with the protective fluxes is similar to that of rare earth metals. In order to obtain the highest possible alloying efficiency it is necessary to use non- $MgCl_2$  fluxes. . . ."

This point of view appeared also to be borne out by a study of the heats of formation of thorium chloride and magnesium chloride. Thus it appears that the heat of formation of thorium chloride is 335,000 cal./mol. compared with 153,300 cal./mol. for magnesium chloride (see Metals Reference Book, Smithells, 1949, pages 434-5). The heat of formation of thorium chloride is therefore over 7,000 cal. higher than that of magnesium chloride per gram equivalent. Accordingly there would appear to be no possibility of removing the rare earth metals from magnesium alloys by magnesium chloride without the simultaneous removal of the thorium.

We have however now carried out a very careful study of the thorium losses from magnesium base alloys and have made the surprising discovery that the losses of thorium which occur on remelting and processing the molten alloys with fluxes containing  $MgCl_2$  are not due to the reaction with magnesium chloride but arise from oxidation, and that the thorium content is not appreciably reduced by treatment even with magnesium chloride alone provided that sufficient care is taken to avoid oxidation. We have further applied this discovery to the possibility of removing rare earth metals from magnesium-thorium alloys with extremely satisfactory results. According to the present invention, therefore, magnesium base alloys containing thorium and one or more rare

## 2

earth metals are intimately contacted with magnesium chloride throughout the body of the alloy while maintaining over the alloy a substance capable of minimising the tendency to oxidation, thereby considerably reducing the rare earth metal content without appreciable reduction of the thorium content. Known means may be employed to minimise oxidation, for example the said substance may be an inert atmosphere such as nitrogen or a suitable flux, or both. A suitable flux is that described in the specification of British patent application No. 5,366/52, for instance:

|          | Percent |
|----------|---------|
| $BaCl_2$ | 40      |
| $MgCl_2$ | 30      |
| KCl      | 10      |
| $CaF_2$  | 20      |

For example an alloy containing 1-4% thorium and 0.2-0.5% rare earth metals may be treated with magnesium chloride thereby reducing the rare earth metal content to less than 0.05% without loss of more than about 0.1% of thorium. In practice the rare earth metal content can be practically completely eliminated without appreciable loss of thorium.

While the invention may be carried out by stirring magnesium chloride, or a mixture of salts containing magnesium chloride, into the molten alloy, we have found that it is preferable to pour the molten alloy into a melt of magnesium chloride or mixture of salts containing magnesium chloride. This salt melt may conveniently be about 2-8% of the weight of the alloy to be treated and moreover the treatment may be repeated two, three or more times. That is to say, the molten alloy may be poured into the molten salt in quantity about 5% of the weight of the alloy and stirred therewith; the molten alloy is then poured into a fresh salt melt of similar quantity, stirred therewith, and then again separated from the salt.

The salt mixture may conveniently consist of magnesium chloride together with potassium chloride. Other salts may also be used such as the chlorides of other alkali metals and alkaline earth metals, and magnesium fluoride may be added to promote a clean separation of metal from flux. Other fluorides however and magnesium oxide should be omitted. In particular  $BaCl_2$  may be added in amounts not less than 15% by weight of the total mixture (e. g. 15 to 50%) in order to avoid introducing persistent chloride contamination in the alloy where the latter contains zirconium in addition to thorium.

We have, therefore, found that it is desirable to carry out this treatment at a comparatively low temperature, e. g. 650° C.-750° C., the removal of rare earth metals being more effective at such temperatures than at higher temperatures. The preferred temperature range is 680° C.-720° C.

As an alternative to the use of  $MgCl_2$  we have found that some removal of rare earth metals from Mg-Th alloys may be effected by bubbling chlorine through the molten alloy, but this process is much less effective.

We claim:

1. A method of reducing the content of rare earth metals in magnesium base alloys containing both thorium and rare earth metals which comprises effecting intimate contact of magnesium chloride with the alloy throughout the body of the alloy, while said alloy is in the molten state, and maintaining over the alloy a substance capable of minimising the tendency of the alloy to oxidation, such substance being selected from the group consisting of metal chloride fluxes, inert atmospheres, and combinations thereof.

2. A method as claimed in claim 1 wherein the alloy

is maintained at a temperature of 650° C. to 750° C. whilst such contact is effected.

3. A method as claimed in claim 1 wherein the alloy is maintained at a temperature of 680° C. to 720° C. whilst such contact is effected.

4. A method as claimed in claim 1 wherein the magnesium chloride is applied to the alloy in admixture with BaCl<sub>2</sub> in quantity at least 15 per cent by weight of the total mixture.

5. A method as claimed in claim 1 wherein the magnesium chloride is applied to the alloy in admixture with at least two other chlorides of the alkali and alkaline earth metals including CaCl<sub>2</sub> in quantity at least 15 per cent by weight of the total mixture.

6. A method as claimed in claim 1 wherein the magnesium chloride is applied to the alloy in admixture with magnesium fluoride and at least two other chlorides of the alkali and alkaline earth metals including BaCl<sub>2</sub> in quantity at least 15 per cent by weight of the total mixture.

7. A method as claimed in claim 1 wherein the molten alloy is poured into a crucible containing molten magnesium chloride, and a further quantity of magnesium chloride is then stirred into the alloy.

8. A method of reducing the content of rare earth metals in magnesium base alloys containing thorium, zirconium and rare earth metals which comprises pouring the molten alloy into a crucible containing a salt mixture in molten condition and subsequently stirring into the alloy a further quantity of such salt mixture, said salt mixture containing at least 25 per cent of magnesium chloride and at least 15 per cent of barium chloride, said mixture being free from magnesium oxide and free from fluorides other than magnesium fluoride, a characteristic of such mixture being that it floats upon the magnesium base alloy and therefore minimizes the tendency of the alloy to oxidation.

References Cited in the file of this patent

UNITED STATES PATENTS

|           |          |               |
|-----------|----------|---------------|
| 2,371,531 | McDonald | Mar. 13, 1945 |
| 2,497,530 | Emley    | Feb. 14, 1950 |
| 2,569,477 | Leontis  | Oct. 2, 1951  |
| 2,604,394 | Emley    | July 22, 1952 |

OTHER REFERENCES

Materials and Methods, February 1946, pages 418-424.  
Journal of Metals, March 1952, pages 287-294.